

Jan. 8, 1952

M. KAHN

2,581,863

PROCESS FOR ELECTRODEPOSITING URANIUM DIOXIDE

Filed March 24, 1945



Fig. 2



Fig. 3



Fig. 1

INVENTOR.  
Milton Kahn  
BY

*Robert A. Gorenstein*  
ATTORNEY

## UNITED STATES PATENT OFFICE

2,581,863

PROCESS FOR ELECTRODEPOSITING  
URANIUM DIOXIDEMilton Kahn, Berkeley, Calif., assignor to the  
United States of America as represented by the  
United States Atomic Energy Commission

Application March 24, 1945, Serial No. 584,686

3 Claims. (Cl. 204—96)

1

This invention relates to the electrolytic deposition of compounds of uranium from aqueous solutions, and more particularly to the electrolytic deposition of insoluble oxides or hydroxides of uranium from aqueous alkaline solutions of ionizing oxycompounds thereof. The invention is especially directed to a process of preparing uranium in a form for isotopic composition analysis. More specifically, the invention appertains to methods and means of preparing compounds of uranium for use in various other instruments and procedures.

It is often necessary to prepare layers of metal or metal compounds for work in which only thin, uniform films can be employed. One such procedure is for the isotopic analysis of metal, such as uranium, as described in the co-pending United States Application Serial Number 536,440 filed May 19, 1944, by Segre and Kennedy, now abandoned. In that method of analyzing polyisotopic uranium, independent measures of mass of sample, and of slow-neutron-produced fission of the sample are required. The last two of these measurements may be made utilizing a target comprising a thin layer of uranous-uranic oxide ( $U_3O_8$ ) on a platinum foil backing. In preparing these targets of uranium for isotopic analysis, it is necessary to prepare the uranium sample as a suitable composition (preferably as substantially pure uranous-uranic oxide) in the form of the film of such thickness that very little alpha particle absorption occurs within the film. A film thickness corresponding to approximately four hundred micrograms of uranium per square centimeter is taken to be about the maximum allowable.

In the prior art process of preparing these target films, chemical methods have generally been employed but considerable difficulty has been encountered in obtaining uniform, thin layers of the desired thickness thereby.

It is an object of this invention to provide methods for improving the Kennedy and Segre method of isotopic analysis, by simplifying the preparation of suitable metal compound films and by eliminating the attendant failures in the prior art methods of film preparation.

It is the further object of this invention to prepare suitable uniform, thin films of metal compounds for use in various procedures by electrodeposition of oxides or hydroxides of uranium.

It is another object of this invention to provide an improved process for preparing a suitably thin film of polyisotopic uranium, whereby the isotopic composition of the uranium may be determined.

2

It is still another object of this invention to provide an improved process of preparing a suitably thin film of purified uranium, as uranous-uranic oxide, whereby the isotopic composition of the uranium may be determined.

Still another object of the invention is to provide a process of electrodepositing a sample of uranium in the form of a film whereby the isotopic composition of the uranium may be determined.

A still further object of the invention is to provide a process for electrodepositing a sample of uranium as a film of uranium dioxide and igniting the uranium dioxide to uranous-uranic oxide, whereby the isotopic composition of the uranium may be determined.

It is an additional object of this invention to provide a process for electrodepositing insoluble uranium oxides or hydroxides from an alkaline solution of a soluble ionizing oxycompound of that metal by reducing the +6 metal ion to the +4 or +3 state whereby the excess hydroxide ions cause a precipitate of the metal oxide or hydroxide.

Other objects and advantages of the invention will appear from the following detailed description including claims and drawings.

In general the present process is directed to the electrolysis of an aqueous alkaline solution of a soluble ionizing oxycompound of uranium so that the +6 metal is reduced at the cathode to the +4 or +3 state and precipitates as the oxide or hydroxide. For example the electrolysis of an alkali metal hydroxide solution of uranyl nitrate (with or without alkali metal carbonate) deposits uranium dioxide on the cathode. This coating may be converted to uranous-uranic oxide by igniting.

By this process oxide or hydroxide films of the order of four hundred micrograms of metal per square centimeter can be prepared. It is preferred to use bright platinized platinum cathodes for preparing heavy films of 250 micrograms per square centimeter or greater.

Additional features and advantages of the present invention will appear from the following detailed description taken in conjunction with the drawing forming part of this specification in which drawing Figure 1 is a vertical section of the electrodeposition cell, Figure 2 is a horizontal sectional view taken on the line 2—2 of Figure 1 showing details of the electrodeposition cell, and Figure 3 shows a conventionalized perspective view with parts out of scale and proportion for clarity of the finished target.

In the drawings a disk 11 which is to be coated with uranium or the like, comprises an approximately 0.002 inch platinum foil cut to a diameter of about one and one-half inches. The disk is thoroughly cleaned, ignited to red heat and tared. The disk is then ready to be assembled as part of the electrodeposition cell 10 in which the disk is to serve as the cathode upon which uranium is to be deposited.

The above-mentioned platinum disk 11 is placed on a larger and thicker platinum disk 12, which is about 0.010 inch in thickness and about two inches in diameter and which is cut so that a tab 13 extends out from the disk and makes connection with the wire 14 to which a negative potential may be applied. In turn, the platinum disk 12 is placed on the ground glass plate 15 which serves as a supporting base for the electrodeposition cell 10. The glass cylinder 16, which is provided with a suitable number (preferably four) of appendant glass hooks 17 and has an outside diameter which is a little less than one and one-half inches, in concentrically placed upon the platinum disk 11 and is secured to this position by passing a band 22 of rubber or the like alternating under the hooks 18 which are arranged in the glass plate 15, as indicated on the drawings, and over the hooks 17 of the glass cylinder 16. A liquid-tight seal is formed at the junction of glass cylinder 18 and platinum disk 11 by forming a fillet 19 of beeswax or the like around the outside of the junction. This is accomplished by applying, with a small brush, molten beeswax to the junction, the beeswax being well above its melting point in order to assure a good seal.

The anode 20 comprises an approximately nine inch length of platinum wire of one-sixteenth diameter of which about six and one-half inches of the length are wound in a spiral leaving about two and one-half inches of straight wire for connection to a stirrer. The platinum anode is fastened in the chuck of the small variable speed electric stirrer, not shown, and the position of this stirrer is adjusted so that the spiral anode dips about half way down into the electrodeposition cell 10. The anode is electrically connected so that it is at a potential positive to that of conductor 14 and is ordinarily grounded. The electrodeposition cell 10 is now completely assembled and is ready for use.

In the case where uranium is to be deposited as uranium dioxide on the platinum disk 11, about ten milliliters of an alkaline carbonate solution (made by adding four grams of potassium carbonate to two hundred milliliters of 0.15 M potassium hydroxide solution thus producing a solution in which the concentration of the carbonate ions and the hydroxyl ions are approximately equal) and about five milliliters of substantially pure uranyl nitrate solution which has been prepared from the uranium sample to be analyzed for isotopic composition are placed in the cell. The concentration of uranyl nitrate solution depends on the amount of uranium which is to be formed as a film on the platinum disk 11. Ordinarily, five milliliters of this solution is made up to contain about two hundred and fifty micrograms of uranium which, when deposited, produces a film of density of about thirty-one micrograms of uranium per square centimeter. The solution, however, may contain as much as about thirty-two hundred micrograms of uranium, in which case, a film of a density of approximately four hundred micro-

grams of uranium per square centimeter is formed when the uranium is deposited. It will thus be apparent that the concentration of carbonate and hydroxide ions will be from about 200 times to 3,000 times the concentration of the uranyl ions. As previously mentioned, such a film is of about the maximum allowable thickness for analytical purposes. A potential of about seven volts is applied to the electrodeposition cell 10, whereby a current of about fifty milliamperes having a current density of about 0.6 ampere per sq. decimeter flows through the cell. At the same time the variable speed electric stirrer (not shown), is turned on, whereby the platinum wire anode 20 is caused to rotate at a suitable speed. The action of the applied potential is to cause the uranium as uranyl ion,  $UO_2^{++}$ , to migrate to the platinum disk 11 and be reduced to a uranous ion,  $U^{4+}$ , which combines with neighboring hydroxyl ions and precipitates as uranium dioxide or, more precisely, as the hydrated dioxide  $UO_2 \cdot 2H_2O$  or the hydroxide  $U(OH)_4$  on the platinum disk 11.

Current is allowed to flow through the electrodeposition cell 10 until the uranium in the cell is substantially completely deposited in a layer 21 on the platinum disk 11. This is accomplished in about ninety minutes. After the current is turned off the solution is poured out of the cell and the cell is rinsed with water. The platinum disk 11 is then detached from the cell and again washed with water. The disk is next ignited in an oxidizing flame for about one minute, whereby any beeswax on the disk is burned off and the exceptionally pure uranium dioxide deposit 21 is quantitatively converted to uranous-uranic oxide,  $U_3O_8$ .

The platinum disk 11, accordingly, is covered with a thin uniform film of  $U_3O_8$  and is ready for the isotopic analysis in accordance with the previously mentioned Segre-Kennedy procedure. This method includes weighing the target, then supporting the target upon a copper base plate and subjecting it to alpha activity and fission activity measurements, whereby both the alpha activity of the  $U_3O_8$  and the fission activity under slow neutron bombardment of the  $U_3O_8$  are determined.

A further example of plating uranium dioxide is to electrolyze in the cell of Figure 1, fifteen c. c. of an aqueous solution containing about 780 micrograms of uranium as uranyl nitrate and about 0.21 gram of potassium hydroxide which provides a hydroxide ion concentration of about 1200 times that of the uranyl ion concentration. A potential of about three volts is applied to the cell whereby a current of about one hundred milliamperes (current density of thirteen milliamperes per square centimeter or 1.3/amps. sq. decimeter) flows therethrough. Current is allowed to flow through the cell until the uranium therein is substantially completely deposited on the platinum disk. This requires about one hundred and sixty minutes. The plated film is treated as in the preceding example. The yield of uranium is checked by weight and by alpha activity and found to be about 90%. The film density is about ninety micrograms per square centimeter.

In view of the foregoing, it is apparent that there has been provided an improved method for preparing uranium in a pure form as a thin film of  $U_3O_8$  in which form the uranium may be analyzed for its isotopic composition. The prep-

aration is accomplished by electrodepositing the uranium as uranium dioxide on a backing member, such as a thin platinum disk, and subsequently igniting the uranium dioxide to  $U_3O_8$ .

The process can be applied to other metals which form soluble higher valence oxycompounds and insoluble lower valence oxides or hydroxides by substituting a corresponding molecular quantity of these metals for the uranium. The ions of such metals should be more susceptible to change in the electrolysis than the anion of the oxycompound and the hydroxyl ions should be in large excess over the metal ion at the cathode in order to have the process effective.

The important factor in this type of electrolysis is to keep the ratio of the concentration in the solution of the uranyl ion to the hydroxyl ion very small so that when the reduced ion (+4 or +3 state) is produced, its rate of diffusion from the cathode will be smaller than the rate of diffusion from the aqueous solution to cathode by the hydroxyl ion. This electrolytic process is to be distinguished from the preparation of films of metal compounds by electrophoresis of colloidal suspensions.

While what has been described is at present considered to be preferred embodiments of the invention, it will be understood that various modifications may be made therein. Thus, for example, backing members of noble metals other than platinum, such as gold, palladium or the like, may be used. Also, for example, soluble salts other than the nitrates, as given in the examples, may be used.

The term uranium, as used in the specifications and claims is used generically to refer to this material whether in elemental or combined state except where indicated otherwise by the context. The term oxide as used in the specification and claims is to include the hydrated oxides or hydroxides unless otherwise indicated by the context.

As many widely different embodiments of this invention may be made without departing from the spirit and scope thereof, it is to be understood that the applicant does not limit himself to the specific disclosures and embodiments except as defined in the appended claims.

What is claimed is:

1. The process for electrodepositing uranium dioxide which comprises contacting two inert electrodes with a dilute aqueous solution wherein

the solute consists essentially of uranyl nitrate and at least one material from the class consisting of potassium carbonate and potassium hydroxide, the amounts of said materials being such that the concentration of the negative ions of said materials is from about 200 times to 3000 times the concentration of the uranyl ion, and passing a direct current through the said solution at a current density of between 0.6 to 1.3 amperes per square decimeter for a period of from about 90 to about 160 minutes.

2. The process of claim 1 wherein the molar concentrations of the carbonate ion and the hydroxyl ion are approximately equal, and current is passed through the solution at a potential of 7 volts and a current density of 0.6 ampere per square decimeter for a period of about 90 minutes.

3. The process for electrodepositing uranium dioxide which comprises contacting two inert electrodes with a dilute aqueous solution wherein the solute consists essentially of uranyl nitrate and potassium hydroxide in amounts such that the molar concentration of the hydroxyl ion is about 1200 times that of the uranyl ion, and passing a direct current through the said solution at a potential of about 3 volts and a current density of about 1.3 amperes per square decimeter for a period of about 160 minutes.

MILTON KAHN.

#### REFERENCES CITED

The following references are of record in the file of this patent:

#### UNITED STATES PATENTS

| Number    | Name           | Date          |
|-----------|----------------|---------------|
| 571,531   | Langhans       | Nov. 17, 1896 |
| 1,448,036 | Pearson et al. | Mar. 13, 1923 |
| 2,059,053 | Stareck        | Oct. 27, 1936 |
| 2,081,121 | Stareck        | May 18, 1937  |

#### OTHER REFERENCES

American Chemical Journal, vol. I, pp. 329-340 (1879).

Journal of American Chemical Society, vol. 29, pp. 806-808 (1907).

Pierle, J. Physical Chemistry, vol. 23, pp. 517-553 (1919).

Handbook of Chemistry and Physics, 26th ed. 1942-1943, page 478, Chemical Rubber Publishing Company.